# EUROPEAN PATENT SPECIFICATION

(11) **EP 1 192 295 B1**
(45) Date of publication and mention of the grant of the patent: **16.11.2005**
(21) Application number: 00930472.6
(22) Date of filing: 08.05.2000
(51) Int. Cl.: C23C 30/00

(54) **ARTICLE EXHIBITING IMPROVED RESISTANCE TO FORMICARY CORROSION**
GEGENSTAND MIT VERBESSERTEM WIDERSTAND GEGEN NESTKORROSION
ARTICLE POSSéDANT UNE RéSISTANCE AMéLIORée à LA CORROSION DU TYPE NID DE FOURMIS

(30) Priority: 01.06.1999 US 324223
(43) Date of publication of application: 03.04.2002
(73) Proprietor: CARRIER CORPORATION, Syracuse, New York 13221 (US)
(72) Inventor: DOWNEY, Sandra, J., Cazenovia, NY 13035 (US); GAROSSHEN, Thomas, J., Glastonbury, CT 06033 (US); GAFFANEY, Daniel, P., Chittenango, NY 13037 (US)
(74) Representative: Leckey, David Herbert
(86) International application number: PCT/US2000/012541
(87) International publication number: WO 2000/073537

(56) References cited:
- PATENT ABSTRACTS OF JAPAN vol. 1996, no. 11, 29 November 1996 (1996-11-29) & JP 08 178585 A (PALOMA IND LTD), 12 July 1996 (1996-07-12)
- PATENT ABSTRACTS OF JAPAN vol. 009, no. 107 (M-378), 11 May 1985 (1985-05-11) & JP 59 229200 A (MATSUSHITA DENKI SANGYO KK), 22 December 1984 (1984-12-22)
- PATENT ABSTRACTS OF JAPAN vol. 1995, no. 09, 31 October 1995 (1995-10-31) & JP 07 166270 A (MITSUBISHI MATERIALS CORP), 27 June 1995 (1995-06-27)
- PATENT ABSTRACTS OF JAPAN vol. 1998, no. 03, 27 February 1998 (1998-02-27) & JP 09 296997 A (KOBE STEEL LTD), 18 November 1997 (1997-11-18)

## Description

This invention relates generally to protecting metals from a corrosive environment, and more specifically, to protecting copper from formicary corrosion when used in a corrosive environment.

Corrosion is a process that involves two simultaneous reactions which are called half-cells. One half-cell reaction is the oxidation or corrosion of the metal. This process involves the loss of electrons, e.g., ${\text{2M →2M}}^{\text{+}} {\text{+2e}}^{\text{-}}$

Electrons from the oxidation process are in tum used by an associated reduction half-cell reaction, which is often the reduction of oxygen or hydrogen, e.g., ${\text{O}}_{\text{2}} {\text{+4H}}^{\text{+}} {\text{+4e}}^{\text{-}} {\text{→ 2H}}_{\text{2}} \text{O}$${\text{2H}}^{\text{+}} {\text{+2e}}^{\text{-}} {\text{→ H}}_{\text{2}}$

The oxidation reaction (corrosion process) can only proceed at a rate governed by the reduction reaction that uses the electrons from the oxidation process. This is because charge neutrality must be maintained.

A unique type of localized corrosion called formicary corrosion, also referred to as ant nest corrosion, occurs in copper when subjected to organic acids in the presence of moisture and air. The result is a rapid tunneling through the copper surface in a random manner, which ultimately leads to through-wall penetration. Prevention of this form of corrosion has typically been accomplished by elimination at least one of the three necessary constituents for its occurence, i.e.., air, moisture, or organic acid However, when at least one of these constituents cannot be removed, as would be the case in an indoor air conditioning application in which an evaporator coil is wet by condensate by virtue of its dehumidification function, alternate protection methods are needed.

There exists a need, therefore, for an improved method of protecting copper in environments which promote formicary corrosion.

JP 08/78585 dicloses a process in which the inner surface of a copper tube is plated with tin. JP 59229200 discloses plating tin, nickel, lead or aluminium ores components of a heat exchanger.

The present invention provides an article as claimed in claim 1.

The primary object of this invention is to provide an article, such as the copper tubes of an evaporator coil, having improved formicary corrosion resistant properties when used in a corrosive environment.

In accordance with a preferred embodiment of this invention, the protective layer comprises a coating formed from one of tin and a tin alloy. Preferably, the coating has a thickness in the range of 0.10 to 1.00 mil (0.0025 to 0.025 mm) and is uniformly applied to the surface. Most preferably, the thickness of the coating is 0.50 mil (0.063 mm)
FIG. 1 is a perspective view of an evaporator coil incorporating copper tubing treated in accordance with the principles of the present invention;
FIG. 2 is a graph illustrating the performance improvements achieved in accordance with the principles of the present invention.

As will be described in detail below, the present invention provides for formicary corrosion protection of copper tubing used in plate-fin coils.

FIG.1 illustrates a plate-fin coil 1 of the type typically used in air conditioning units. The coil includes one or more flow circuits for carrying refrigerant therethrough. For the purposes of explanation, the coil 1 contains a single flow circuit tube 2 consisting of an inlet line 3 and an outlet line 4, and a plurality of fins 5 extending radially therefrom.

As noted above, evaporator coils of this type are commonly used in corrosive environments. In a typical arrangement, coils of this type are fabricated utilizing copper tubing for the circuit flow tubes. Copper is utilized in tube construction because of its good heat transfer properties, general resistance to corrosion, and ease of fabrication and repair.

In accordance with the principles of the present invention, the exposed surface of the copper tube 2 is coated or enriched with a material for preventing formicary corrosion. Tin and tin alloys are the best candidates for this material. Thus, substantial improvements in the resistance to formicary corrosion is achieved by coating or impregnating the copper tubing's surface with a layer of material such as tin or tin alloy.

The improvement achieved using the principles of the present invention is illustrated graphically in FIG. 2. Testing has shown a greater than twenty fold (20x) improvement in the failure rate of copper when, for example, copper tubing is coated with 0.5 mil (0.063 mm) of electroplated tin. Other methods of prevention such as using formicary corrosion inhibitors (not including removing one of the three factors causing formicary corrosion which is rarely a feasible option), typically show only a three fold (3x) improvement. Accordingly, by coating the formicary corrosion susceptible copper tubing with a metal that is resistant to such corrosion, the corrosion resistance of the copper tubing is significantly improved. While pure tin is the preferred material, tin alloys containing such metals as zinc, magnesium, copper, gallium, cadmium and lead will also result in improved resistance to formicary corrosion of the copper. Other metals also increasing the resistance to formicary corrosion may be used as well.

The coating or surface enrichment of the copper tubes 2, in the embodiment illustrated, with tin or other discussed material is accomplished prior to the assembly of the heat exchanger 10. There are several methods for applying the protective coating systems to copper tubing. Potential methods include: (1) hot dipping, (2) electroplating (3) vapor deposition, and (4) ion implantation.

This invention includes all coatings that work to prevent formicary corrosion of copper. The proposed approach is very cost effective and maintains the thermal conduction of the copper tubing in heat exchanger applications. High thermal conduction is accomplished by using a coating with a relatively high thermal conductivity or by applying very thin coatings.

An important aspect of the present invention is the production of a uniform coating of formicary corrosion reaction resistant material over the entire exterior surface of the flow circuit tubes 2. Regardless of the process used, the variables of tube surface preparation, tube preheat temperature, coating composition, and coating thickness need to be carefully controlled to achieve the proper results of the present invention. The preparation of the exposed surfaces of the tube is designed to remove the surface oxide layer from the copper to ensure that the coating material will adhere well to the tube. A number of surface preparation processes are known in industry and include the use of acid reducing gases, fluxes and mechanical abrasion such as shot blasting It is preferred that the coating have high ductility to allow for the subsequent assembly of the heat exchanger without damaging the coating. The ductility of the coating is determined in part by the coating composition and the thickness of the coating. The coating must be thick enough to prevent the penetration of the electrolyte, and thin enough to have good formability and cost benefits. The optimal range of thickness is 0.10 mils to 1.0 mils (0.0025 to 0.025 mm)

The primary advantage of this invention is that an article is provided, such as a plate-fin heat exchanger coil, having improved formicary corrosion resistant properties when used in a corrosive environment. Another advantage of this invention is that a copper tube evaporator is provided having a coating for inhibiting corrosion activities due to formicary corrosion. Yet another advantage of this invention is that a plate-fin coil is provided formed from copper tubing with a tin or tin alloy coating for inhibiting formicary corrosion.

## Claims

1. An article resistant to formicary corrosion comprising a flow circuit tube (2) made from copper, said tube having a refrigerant inlet (3) and a refrigerant outlet (4), and further comprising a plurality of fins (5) connected to, and extending radially from, the tube (2), the external surface of said tube (2) having a layer provided on its surface for preventing formicary corrosion of the tube, **characterised in that** said layer extends under the fins (5) between the fins (5) and the tube (2).

2. An article according to claim 1 wherein the layer comprises a coating on the surface, said coating being of a metal that has a greater resistance to formicary corrosion than does copper.

3. An article according to claim 1 or 2 wherein said coating is applied uniformly to said surface.

4. An article according to claim 3 wherein the coating has a thickness in the range 0.10 to 1.00 mil (0.0025 to 0.025 mm).

5. An article according to claim 1 wherein said layer is a coating comprising one of tin and a tin alloy.

6. An article according to claim 5 wherein the coating has a thickness in the range 0.10 to 1.00 mil (0.0025 to 0.025 mm) .

7. An article according to claim 1 wherein said layer is a tin coating having a uniform thickness of about 0.5 mil (0.0063 mm) .

8. A method of protecting from formicary corrosion an article which comprises a flow circuit tube (2) made from copper, said tube having a refrigerant inlet (3) and a refrigerant outlet (4), and a plurality of fins (5) connected to and extending radially from the tube (2) comprising the steps of:
providing on the external surface of said tube, prior to the attachment of the fins thereto, a layer which is resistant to formicary corrosion.

9. A method according to claim 8 wherein the layer comprises a coating on the surface, said coating being of a metal that has a greater resistance to formicary corrosion than does copper.

10. A method according to claim 8 or 9 wherein said coating is applied uniformly to said surface.

11. A method according to claim 10 wherein the coating has a thickness in the range 0.10 to 1.00 mil (0.0025 to 0.025 mm) .

12. A method according to claim 8 wherein said layer is a coating comprising one of tin and a tin alloy.

13. A method according to claim 12 wherein the coating has a thickness in the range 0.10 to 1.00 mil (0.0025 to 0.025 mm).

14. A method according to claim 8 wherein said layer is a tin coating having a uniform thickness of about 0.5 mil (0.0063 mm) .

## Patentansprüche

1. Gegenstand, der widerstandsfähig gegen Ameisennestkorrosion ist, aufweisend ein aus Kupfer gebildetes Strömungskreisrohr (2), wobei das Rohr einen Kühlmitteleinlass (3) und einen Kühlmittelauslass (4) hat, und ferner aufweisend eine Mehrzahl von Lamellen (5), die mit dem Rohr (2) verbunden sind und von diesem radial weg ragen, wobei die Außenoberfläche des Rohrs (2) eine an ihrer Oberfläche vorgesehene Schicht zum Vermeiden von Ameisennestkorrosion des Rohrs aufweist,
**dadurch gekennzeichnet, dass** sich die Schicht unter den Lamellen (5), zwischen den Lamellen (5) und dem Rohr (2) erstreckt.

2. Gegenstand nach Anspruch 1, wobei die Schicht eine Beschichtung an der Oberfläche aufweist, wobei die Beschichtung aus einem Metall ist, das eine größere Widerstandsfähigkeit gegen Ameisennestkorrosion aufweist als Kupfer.

3. Gegenstand nach Anspruch 1 oder 2, wobei die Beschichtung gleichmäßig auf die Oberfläche aufgebracht ist.

4. Gegenstand nach Anspruch 3, wobei die Beschichtung eine Dicke im Bereich von 0,10 bis 1,00 Mil (0,0025 bis 0,025 mm) hat.

5. Gegenstand nach Anspruch 1, wobei die Schicht eine Beschichtung ist, die entweder Zinn oder eine Zinnlegierung aufweist.

6. Gegenstand nach Anspruch 5, wobei die Beschichtung eine Dicke im Bereich von 0,10 bis 1,00 Mil (0,0025 bis 0,025 mm) aufweist.

7. Gegenstand nach Anspruch 1, wobei die Schicht eine Zinnbeschichtung mit einer gleichmäßigen Dicke von etwa 0,5 Mil (0,0063 mm) ist.

8. Verfahren zum Schützen eines Artikels, der ein aus Kupfer gebildetes Strömungskreisrohr (2) aufweist, gegen Ameisennestkorrosion, wobei das Rohr einen Kühlmitteleinlass (3) und einen Kühlmittelauslass (4) und eine Mehrzahl von Lamellen (5), die mit dem Rohr (2) verbunden sind und sich von diesem radial erstrecken, aufweisend die Schritte:
Versehen der Außenoberfläche des Rohrs, vor dem Anbringen der Lamellen daran, mit einer Schicht, die gegen Ameisennestkorrosion widerstandsfähig ist.

9. Verfahren nach Anspruch 8, wobei die Schicht eine Beschichtung an der Oberfläche aufweist, wobei die Beschichtung aus einem Metall ist, das eine größere Widerstandsfähigkeit gegen Ameisennestkorrosion aufweist als Kupfer.

10. Verfahren nach Anspruch 8 oder 9, wobei die Beschichtung gleichmäßig auf die Oberfläche aufgebracht wird.

11. Verfahren nach Anspruch 10, wobei die Beschichtung eine Dicke im Bereich von 0,10 bis 1,00 Mil (0,0025 bis 0,025 mm) hat.

12. Verfahren nach Anspruch 8, wobei die Schicht eine Beschichtung ist, die entweder Zinn oder eine Zinnlegierung aufweist.

13. Verfahren nach Anspruch 12, wobei die Beschichtung eine Dicke im Bereich von 0,10 bis 1,00 Mil (0,0025 bis 0,025 mm) hat.

14. Verfahren nach Anspruch 8, wobei die Schicht eine Zinnbeschichtung mit einer gleichmäßigen Dicke von etwa 0,5 Mil (0,0063 mm) ist.

## Revendications

1. Article résistant à une corrosion en nid de fourmis comprenant un tube (2) de circuit d'écoulement en cuivre, ledit tube ayant un orifice d'entrée (3) pour réfrigérant et un orifice de sortie (4) pour réfrigérant, comprenant en outre une pluralité d'ailettes (5) connectées à, et s'étendant radialement depuis, le tube (2), la surface externe dudit tube (2) portant une couche de surface pour empêcher une corrosion en nid de fourmis du tube, **caractérisé en ce que** ladite couche s'étend sous les ailettes (5) entre les ailettes (5) et le tube (2).

2. Article selon la revendication 1 dans lequel la couche comprend un revêtement de surface, ledit revêtement étant en un métal qui a une résistance plus importante à une corrosion en nid de fourmis que le cuivre.

3. Article selon la revendication 1 ou 2, dans lequel ledit revêtement est appliqué uniformément sur ladite surface.

4. Article selon la revendication 3, dans lequel le revêtement a une épaisseur comprise dans la plage allant de 0,10 à 1,00 mil (0,0025 à 0,025 mm).

5. Article selon la revendication 1, dans lequel ladite couche est un revêtement comprenant de l'étain ou un alliage d'étain.

6. Article selon la revendication 5, dans lequel le revêtement a une épaisseur comprise dans la plage allant de 0,10 à 1,00 mil (0,0025 à 0,025 mm).

7. Article selon la revendication 1, dans lequel ladite couche est un revêtement en étain ayant une épaisseur uniforme d'environ 0,5 mil (0,0063 mm).

8. Procédé de protection d'une corrosion en nid de fourmis d'un article qui comprend un tube (2) de circuit d'écoulement en cuivre, ledit tube ayant un orifice d'entrée (3) pour réfrigérant et un orifice de sortie (4) pour réfrigérant, et une pluralité d'ailettes (5) connectées à et s'étendant radialement depuis le tube (2), comprenant les étapes consistant à :
déposer sur la surface externe dudit tube, avant de fixer les ailettes sur ce dernier, une couche qui est résistante à une corrosion en nid de fourmis.

9. Procédé selon la revendication 8, dans lequel la couche comprend un revêtement de surface, ledit revêtement étant en un métal qui a une résistance plus importante à une corrosion en nid de fourmis que le cuivre.

10. Procédé selon la revendication 8 ou 9, dans lequel ledit revêtement est appliqué uniformément sur ladite surface.

11. Procédé selon la revendication 10, dans lequel le revêtement a une épaisseur comprise dans la plage allant de 0,10 à 1,00 mil (0,0025 à 0,025 mm).

12. Procédé selon la revendication 8, dans lequel ladite couche est un revêtement comprenant de l'étain ou un alliage d'étain.

13. Procédé selon la revendication 12, dans lequel le revêtement a une épaisseur comprise dans la plage allant de 0,10 à 1,00 mil (0,0025 à 0,025 mm).

14. Procédé selon la revendication 8, dans lequel ladite couche est un revêtement d'étain ayant une épaisseur uniforme d'environ 0,5 mil (0,0063 mm).
